

[54] **METHOD FOR PRINTING TEXTILES USING A PRECOAT CONTAINING  $\beta$ -1,4 GLUCAN**

[75] Inventors: **Noriaki Mizuma, Tokyo; Yuzo Yokota, Oi-Machi, both of Japan**

[73] Assignee: **FMC Corporation, Philadelphia, Pa.**

[\*] Notice: The portion of the term of this patent subsequent to July 25, 1989, has been disclaimed.

[22] Filed: **Feb. 7, 1972**

[21] Appl. No.: **224,246**

**Related U.S. Application Data**

[63] Continuation-in-part of Ser. No. 28,144, April 13, 1970, abandoned.

[52] **U.S. Cl..... 8/62; 8/91**

[51] **Int. Cl..... D06p 1/48**

[58] **Field of Search..... 8/91, 62, 167**

[56] **References Cited**

**UNITED STATES PATENTS**

1,884,620 10/1932 Dreyfus..... 8/167

|           |         |                |      |
|-----------|---------|----------------|------|
| 3,259,537 | 7/1966  | Battesta ..... | 8/   |
| 3,485,572 | 12/1969 | Taube .....    | 8/62 |
| 3,679,352 | 7/1972  | Mizuma .....   | 8/83 |

**OTHER PUBLICATIONS**

Exporte Weissbein, Paper No. 18, in Patent File of Pat. No. 3,679,351, 4 pages with 4 pages attachment listing discontinued dyes.

*Primary Examiner*—Donald Levy

[57]

**ABSTRACT**

Pre-treating of textile fabrics with an aqueous dispersion of finely-divided  $\beta$ -1,4 glucan particles and a water-soluble binder to provide sharper and deeper colored prints from a printing process which employs a steam treatment.

**3 Claims, No Drawings**

**METHOD FOR PRINTING TEXTILES USING A  
PRECOAT CONTAINING  $\beta$ -1,4 GLUCAN**

This application is a continuation-in-part of copending application Ser. No. 28,144, filed Apr. 13, 1970 now abandoned.

This invention relates to a method for the treatment of textile fabrics prior to printing, especially fabrics of hydrophobic fibers, synthetic fibers and fabrics of blends of hydrophobic and hydrophilic fibers, to improve sharpness, uniformity and color yield for dyeing.

In order to keep pace with developments in the synthetic fiber industry and the marked progress of techniques of their fiber blending and weaving, there is an urgent need for improvement in the printing art and studies of all aspects thereof are being made. Nevertheless, under the present state of conditions where there are infinite varieties of print material and the requirements for printability have become more and more exacting, many unsolved problems remain. It is a known fact that the improvement of color printing characteristics including sharpness of "bleeding", uneven printing and color yield are urgent problems. It has heretofore been known that, in hydrophobic articles such as in synthetic fibers or their blended or mixed fabrics, lack of affinity between aqueous dye-paste and fabrics for printing produces a serious drawback at the time of printing and especially steaming. Excess water in the dye-paste floats on the surface of the textile fabric, causing a capillary phenomenon, externally moving out of the printed pattern, and thus producing bleeding. Furthermore, such excess of water, upon being subjected to printing pressure from rollers or squeezers, easily reaches to the back of the fabric. And, as a result of such osmosis, not only is there uneven dyeing, but also less residual adhesion of dye-paste on the fabric, thus deteriorating color yield.

It has now been discovered that the above printing defects may be substantially overcome and high printability secured with a specific pre-treatment for textile fabric to be printed.

The method of this invention comprises coating a textile fabric with an aqueous dispersion consisting essentially of finely-divided, water-insoluble organic particles at least about 90 percent, preferably 99 percent by weight consisting of  $\beta$ -1,4 glucan and a water-soluble binder, drying said coating, printing a design on said fabric with a colored printing paste, treating the printed textile with direct application of steam, washing the textile to remove said organic particles and drying the textile.

This is an improvement over the disclosure of U.S. Pat. No. 3,259,537 to Orlando A. Battista.

The water-insoluble, organic material is originally derived from cellulose-containing plant life, in most instances, wood, cotton, and bast or leaf fibers. In general, materials obtained from a holo-cellulose source are most useful, for example, ramie, flax, hemp, cotton, processed cellulose-containing material, for example, cotton linters, purified cotton, wood pulps such as bleached sulfite and sulfate pulps, regenerated forms of cellulose including rayon and cellophane, and the like. If the source material is too low in  $\beta$ -1,4 glucan content, it is purified to remove nonessential or undesirable components such as pentosans, galactomannans, glucomannans, and the like, to provide a product con-

taining at least 90 and preferably at least about 99 percent of  $\beta$ -1,4 glucan.

The method of achieving the low particle size is not critical from the standpoint of this invention and will generally include, for example, mechanical disintegration, a combination of chemical degradation and mechanical attrition, chemical treatment only, precipitation from solution, and chemical regeneration. It is preferred on the basis of practical utility, that a combination of chemical degradation and mechanical attrition be used in forming the specified particulate size of the water-insoluble  $\beta$ -1,4 glucan-containing material.

Hereinafter, the term "cellulose" will be used to represent  $\beta$ -1,4 glucan-containing materials for ease of explanation and illustration.

Chemical degradation of the cellulose material is brought about in a known manner to facilitate disintegration, for example, the material may be subjected to acid or alkali hydrolysis, or enzymatic treatment. One specific method of obtaining the desired result is reported in U.S. Pat. No. 2,978,446, issued Apr. 4, 1961, to Orlando A. Battista et al, wherein cellulose is subjected to a 2.5 normal aqueous solution of hydrochloric acid at boiling (about 105°C.) for 15 minutes. This more drastic hydrolysis treatment provides a material which may be readily mechanically attrited in an aqueous medium with a nominal amount of energy. Similar treatments with mineral acids or alkali under more or less drastic conditions will produce attritable degraded cellulose using nominal or increased energy for disintegration of the material to the proper particle size.

The type of starting material prior to chemical degradation will also determine the amount or input energy for attrition of the cellulose to obtain the desired particle size. For example, dilute hydrochloric acid hydrolysis of regenerated forms of cellulose will produce a material substantially all of which can be attrited to the desired particle size by merely dispersing the same with a conventional electrically driven kitchen beater in an aqueous medium for a few minutes. Other forms of cellulose, for example, wood pulp and cotton linters, after a similar hydrolysis treatment must be attrited with the same or more efficient equipment for at least one half hour or more in an aqueous medium to provide a material at least a portion of which is within the desired particle size range. Mechanical attrition may be carried out by known techniques using for example, kitchen mixers, blenders, planetary mixers, ball mills, attrition mills, sonic mixers, high speed shearing devices and the like. In addition, the material may be forced through a multiplicity of fine holes whereby it is subjected to a shearing action first by passage through said holes and thereafter by rubbing together of the various particles under the influence of applied force. The disintegration is preferably carried out in the presence of an aqueous medium to appreciably reduce the energy necessary to produce smaller particle sizes. The attrition should be extended to produce a mass wherein at least 30 percent of the particles are less than 1 micron and preferably over 80 percent of the particles measure no greater than about 0.4 micron. Particles having a size, for example, as small as 0.01 micron are useful for this invention.

As previously stated, regenerated forms of cellulose, for example, regenerated cellulose film, are easily brought to the prescribed particle size after the controlled acid hydrolysis by merely dispersing the wet-

cake material in water with a mixer. This will produce a stable dispersion wherein the dispersed particles are substantially all less than the prescribed 0.4 micron size. When wood pulp, cotton linters, and similar cellulose materials of greater molecular weight are hydrolyzed under controlled conditions and mechanically attrited in an aqueous medium, many larger particles are present along with the desired small particles. When these cellulosic materials are dried after attrition they are difficult to redisperse in water. It has been found that this type of material may be advantageously combined with a minor proportion of a specific barrier material to provide a readily redispersible mass.

Briefly, the barrier material is a specified sodium salt of carboxymethyl cellulose having a degree of substitution of from about 0.60 to about 0.90, and preferably having a viscosity in centipoises at 25°C. in a 2 percent aqueous solution of less than 18 up to about 800. The barrier may be combined with the finely-divided cellulose by drying a suspension of the cellulose particles in the presence of about 5 to 15 percent of the barrier material. The combination of barrier and cellulose particles is effective for the purpose of this invention.

The finely-divided material can be used in its originally dispersed form or it may be dried to a powdery material for example, by air or spray drying techniques and then redispersed.

When the finely-divided cellulose is dried, e.g. by spray drying, it tends to agglomerate into larger particle sizes in the range of 50-100 microns and greater. To redisperse this material in water, if it has not been combined with CMC as disclosed above, high shear or mixing energy must be used.

An aqueous dispersion of this finely-divided cellulose is coated on textile cloth for printing employing a suitable method such as padding, coating, spraying, etc. in the presence such as water-soluble high polymer, e.g. polyvinyl alcohol, rice starch, wheat starch, natural gums, artificial gums, e.g. the sodium salt of carboxymethyl cellulose, or mixtures of these in an amount preferably ranging from about 0.5 to about 5 percent based on the weight of the aqueous dispersion. The textile is then dried and put to printing. In this case, the addition of finely-divided cellulose to the textile is in an amount sufficient to improve sharpness of printing thereon after a direct application of steam thereto, preferably from about 1 to about 10 percent based on the weight of the aqueous dispersion. The pre-treated cloth fabric thus obtained has suitable water absorbency and water retention mainly on its surface layer, absorbing any excess of water in the dye-paste and further preventing capillary phenomenon. Consequently, it is possible to develop in an exact manner a clear pattern having excellent sharpness by holding down bleeding, as well as providing uniform printing without uneven dyeing. Furthermore, there is no limitation in the application of this printing method to any of the known printing processes such as hand printing, roll printing, screen printing and so forth, which set the printing on the fabric by direct application of steam, e.g. at 100°-150°C. for a few minutes up to an hour. Since the coating of finely-divided cellulose comes off cloth surfaces easily by ordinary washing, the practical value is high without causing any trouble in appearance or texture of the textile fabric.

The invention is further illustrated by means of examples as follows:

## EXAMPLE I

To 100 parts of water were added wheat starch, polyvinyl alcohol and finely-divided cellulose in a ratio indicated in Table I, and the mixture was fully mixed and agitated to give four types of treating solutions. The finely-divided cellulose was prepared by the acid hydrolysis and attrition of wood pulp to obtain a product dispersed in an aqueous medium wherein all of the cellulose particles were less than 1 micron. This dispersion of finely-divided cellulose containing 10 percent of a CMC having a D.S. of 0.75 was spray dried to obtain a powdery substance having an average particle size of 80-90 microns. Polyester textile fabrics were dipped in each solution, pressed between rolls at roll pressure of 2 kg/cm<sup>2</sup>, then dried for 2.5 minutes on a pin tenter at 105°C. Thus, pretreatment was effected.

Next, using a standard type screen having gauze of 95 mesh, the aforementioned pre-treated fabrics were color printed with a printing paste using a screen process, air-dried, heated by direct application of steam for 20 minutes and, after washing with water, scoured for finishing. For comparison's sake, the same fabric, not having been subjected to the pre-treatment process, was printed and after-treated in an identical manner.

The printing paste used for this screen printing had the following composition:

|                                     |   |            |
|-------------------------------------|---|------------|
| Dye — Color Index, Disperse Blue 98 | — | 15 grams   |
| Thickener — Locust bean gum         | — | 20 grams   |
| Solubilizer — Thioethylene glycol   | — | 2 grams    |
| Water                               | — | 963 grams  |
| TOTAL                               |   | 1000 grams |

In Table II and the following examples, the sharpness of printing is represented by the height of a blank triangle reproduced by printing using a standard 95 mesh screen, the original triangle pattern having dimension of 0.3 cm. along the base and 10 cm. in height. A greater height of the reproduced triangle indicates better sharpness, the best sharpness being represented by a measurement of 95 mm. for the printed triangle. The dye bleeding after printing and direct steaming is determined by the length of the base of the above-mentioned triangle. Accordingly, a greater length of the base indicates a greater degree of bleeding. The optimum bleeding condition is represented by a measurement of 2.7 mm. for the base of the printed triangle.

TABLE I

| Treating Solution | Wheat starch (parts) | PVA (parts) | Cellulose crystallite aggregates (parts) |
|-------------------|----------------------|-------------|------------------------------------------|
| A                 | 2                    | 0           | 0                                        |
| B                 | 1                    | 2           | 2                                        |
| C                 | 2                    | 2           | 4                                        |
| D                 | 0                    | 4           | 6                                        |

TABLE II

|                       | Sharpness (mm) | Bleeding (mm) | Even dyeing printability | Color Yield  |
|-----------------------|----------------|---------------|--------------------------|--------------|
| Non-pre-treated cloth | 78             | 4.5           | poor                     | lightly dyed |
| Pre-treated cloth     |                |               |                          |              |

TABLE II-Continued

|                   | Sharpness<br>(mm) | Bleeding<br>(mm) | Even dyeing<br>printability | Color<br>Yield        |
|-------------------|-------------------|------------------|-----------------------------|-----------------------|
| with A solution   | 81                | 4.5              | poor                        | lightly dyed          |
| Pre-treated cloth |                   |                  |                             |                       |
| with B solution   | 87                | 3.3              | good                        | slightly<br>deep dyed |
| Pre-treated cloth |                   |                  |                             |                       |
| with C solution   | 89                | 3.2              | good                        | deeply dyed           |
| Pre-treated cloth |                   |                  |                             |                       |
| with D solution   | 89                | 3.2              | good                        | deeply dyed           |

## EXAMPLE II

A solution (treating solution E) consisting of two parts of polyvinyl alcohol added to 100 parts of water and another dispersed solution (treating solution F) consisting of 10 parts of finely-divided cellulose added to treating solution E were prepared.

The finely-divided cellulose was prepared by the acid hydrolysis and attrition of regenerated cellulose waste to obtain a product dispersed in an aqueous medium wherein 66 percent of the cellulose particles were under 0.2 micron and substantially all of the remainder were under 1 micron. This dispersion was spray dried to provide a powdery substance having an average particle size of 50-75 microns. Using a roll coating machine, nylon fabrics were coated with each solution and dried for 2.5 minutes on a pin tenter, thereafter given to printing in a similar manner as described in Example I except that the printing paste had the following composition.

|                                   |       |            |
|-----------------------------------|-------|------------|
| Dye — Color Index, Acid Red 117   | —     | 15 grams   |
| Thickener — Locust bean gum       | —     | 15 grams   |
| Solubilizer — Urea                | —     | 2 grams    |
| Acid generator — Ammonium sulfate | —     | 5 grams    |
| Water                             | —     | 963 grams  |
|                                   | TOTAL | 1000 grams |

The result is observed with naked eyes, judged, and indicated in Table III. For comparison's sake, printing was made on a cloth not subjected to pre-treatment.

TABLE III

|                                               | Sharpness<br>(mm) | Bleeding<br>(mm) | Color Yield<br>(%) |
|-----------------------------------------------|-------------------|------------------|--------------------|
| Non-pre-treated cloth                         | 75                | 4.3              | 55                 |
| Pre-treated cloth with<br>treating solution E | 79                | 4.3              | 51                 |
| Pre-treated cloth with<br>treating solution F | 90                | 3.5              | 43                 |

Color yield referred to in the table above means the measurement of transparency determined by first cutting a given quantity of printed part of each sample, extracting with pyridine solution, and measuring the transparency of extract solution with a photoelectric photometer. Thus, greater the value, the lower the color yield. The same applies hereafter.

## EXAMPLE III

Mixed with 100 parts of water were sodium salt of carboxymethyl cellulose (CMC) and cellulose crystallite aggregates in a ratio indicated in Table IV, then agitated to provide a treating solution. Following the pre-

treatment of nylon fabric with said treating solution similarly as done in Example I, the nylon fabric was printed with a printing paste similar to that of Example II, using a roll printer, air-dried, heated by direct application of steam, washed and scoured. The results shown in Tables V and VI reveal excellent even printing.

TABLE IV

| Treating<br>solution | CMC<br>(parts) | Cellulose crystalline<br>aggregate (parts) |   |
|----------------------|----------------|--------------------------------------------|---|
|                      |                | G                                          | H |
| I                    | 2              | 0                                          | 2 |
| J                    | 2              | 4                                          | 6 |

TABLE V

|                                               | Sharp-<br>ness   | Bleeding                         | Even<br>print-<br>ability | Color<br>Yield  |
|-----------------------------------------------|------------------|----------------------------------|---------------------------|-----------------|
| Non-pre-treated cloth                         | poor             | poor                             | uneven                    | lightly<br>dyed |
| Pre-treated cloth with<br>treating solution G | poor             | Marked bleed-<br>ing in steaming | uneven                    | lightly<br>dyed |
| Pre-treated cloth with<br>treating solution H | slightly<br>poor | good                             | good                      | deeply<br>dyed  |
| Pre-treated cloth with<br>treating solution I | good             | very<br>good                     | good                      | deeply<br>dyed  |
| Pre-treated cloth with<br>treating solution J | good             | good                             | good                      | deeply<br>dyed  |

TABLE VI

|                                               | Sharpness<br>(mm) | Bleeding<br>(mm) | Color<br>Yield<br>(%) |
|-----------------------------------------------|-------------------|------------------|-----------------------|
| Non-pre-treated cloth                         | 79                | 4.2              | 48                    |
| Pre-treated cloth with<br>treating solution G | 78                | 4.3              | 52                    |
| Pre-treated cloth with<br>treating solution H | 85                | 3.4              | 42                    |
| Pre-treated cloth with<br>treating solution I | 88                | 3.1              | 41                    |
| Pre-treated cloth with<br>treating solution J | 88                | 3.2              | 41                    |

The above two tables show that the use of a water-soluble polymer alone such as CMC does not improve the print pattern as compared to the non-pre-treated cloth while the combination of the water-soluble polymer and the finely-divided cellulose give great improvement.

Various changes and modifications may be made practicing this invention without departing from the spirit and scope thereof and therefore the invention is not to be limited except as defined in the appended claims.

We claim:

1. A method of printing textile fabric which comprises coating said textile fabric with an aqueous dispersion consisting essentially of finely-divided, water-insoluble organic particles at least about 90 percent by weight consisting of  $\beta$ -1,4 glucan and a water-soluble binder, drying said coating, printing a design on said fabric with a colored printing paste, treating the printed textile with the direct application of steam, washing the textile to remove the dried coating and drying the textile.

2. The method of claim 1 wherein the finely-divided organic particles are present in the aqueous dispersion in an amount ranging from about 1 to 10 percent based on the weight of the dispersion and the water-soluble binder is present in an amount ranging from about 0.5

5

to 5 percent based on the weight of the dispersion.

3. The process of claim 1 wherein the textile fabric comprises hydrophobic fibers.

\* \* \* \* \*

10

15

20

25

30

35

40

45

50

55

60

65

UNITED STATES PATENT OFFICE  
CERTIFICATE OF CORRECTION

PATENT NO. : 3,897,204

DATED : July 29, 1975

INVENTOR(S) : Noriaki Mizuma and Yuzo Yokota

It is certified that error appears in the above-identified patent and that said Letters Patent are hereby corrected as shown below:

Col. 1, line 41, "specific" should read --specified--.

Col. 2, line 13, "tern" should read --term--;

line 58, "hwherein" should read --wherein--.

**Signed and Sealed this**  
***second Day of December 1975***

[SEAL]

*Attest:*

**RUTH C. MASON**  
*Attesting Officer*

**C. MARSHALL DANN**  
*Commissioner of Patents and Trademarks*